

# UNITED STATES PATENT OFFICE.

ROBERT D. PIKE, OF SAN FRANCISCO, CALIFORNIA.

## CARBON ELECTRODE AND METHOD OF MANUFACTURING SAME.

1,215,700.

Specification of Letters Patent. Patented Feb. 13, 1917.

No Drawing.

Application filed March 13, 1916. Serial No. 83,766.

To all whom it may concern:

Be it known that I, ROBERT D. PIKE, a citizen of the United States, residing in the city and county of San Francisco and 5 State of California, have invented certain new and useful Improvements in Carbon Electrodes and Methods of Manufacturing Same, of which the following is a specification.

10 The present invention relates to carbon electrodes mainly designed for use in electro-chemical industries and in dry batteries, and the invention resides in the production of carbons for use generally from what is 15 commonly known as "lamp black" refuse derived from the manufacture of illuminating gas from petroleum.

I have discovered that carbons produced from the so-called "lamp black" refuse from 20 the manufacture of illuminating gas from petroleum possess certain qualities lacking in the ordinary carbon electrodes, noticeably a denser structure freer from porosity and a higher degree of electric conductivity.

25 The former feature is not possessed by any other carbon electrodes made from materials as cheap as this refuse "lamp black" and the latter quality namely of electric conductivity is not possessed in such high 30 degree by any other carbon electrodes used for these purposes. These qualities are of advantage, in that less of the material being treated is absorbed by a dense carbon than by a porous carbon and there is less tendency for the carbon to disintegrate and the 35 higher electric conductivity enables more electricity to be conducted to the work for a given weight of electrode. Inasmuch as refuse "lamp black" is a very cheap by-product 40 produced in great abundance wherever illuminating gas is manufactured from petroleum, as in California and Oregon, I am able to produce electrodes of superior quality at a very low cost.

45 By the term "lamp black" refuse as employed herein is not meant "lamp black" in the true sense commonly employed, *i. e.* finely divided carbon deposited from smoke or smoky flame. On the contrary, the "lamp 50 black" refuse from gas plants is neither a true "lamp black" nor a true coke, but, in reality, is a distinct form of amorphous carbon, being just as distinct from either the "coke" or true "lamp black" as these two 55 latter differ from each other.

True "lamp black" is a product contain-

ing no impurities; as produced it is practically pure carbon. It is this form of lamp black which has heretofore been employed in connection with the manufacture of electrodes and carbons.

Refuse "lamp black" is one of the by-products derived from the manufacture of illuminating gas from petroleum, and the manner of its production is, in brief, the spraying of petroleum, air and steam upon red hot fire bricks in an inclosed space or chamber, resulting in a molecular re-arrangement, and the consequent production of illuminating gas, tar and refuse "lamp black"; the last named is separated from the gas by passage through cold water. The temperature of its formation is high, the gases carrying the refuse "lamp black" in suspension having a temperature of approximately 1800 degrees Fahr., before plunging into the cooling water which precipitates the so-called "lamp black". This so-called refuse "lamp black" is gritty and when dried and purified is a steel gray color, and when 75 examined under a high power microscope discloses a different characteristic structure of particles from true "lamp black". The name "lamp black" as indicating a refuse by-product from gas manufacturing plants, 80 is employed by those connected with the manufacture of gas to designate such by-product for lack of a more expressive term. True "lamp black" is lighter in weight; the weight of a cubic inch of true "lamp black" 85 is about  $\frac{1}{6}$  of an ounce, whereas the weight of a cubic inch of refuse "lamp black", after being purified and dried, is about .42 oz.

I have found that the so-called "lamp black" refuse from the manufacture of illuminating gas from petroleum, per hundred pounds contains the following in about the proportions given:

Three pounds of soluble and insoluble ash, of which two and one-half pounds is soluble:—

|                                           |            |
|-------------------------------------------|------------|
| Tar                                       | 30 pounds. |
| Hydrocarbons, volatile at low temperature | 10 pounds. |
| Water                                     | 30 pounds. |
| "Lamp black"                              | 27 pounds. |

In carrying out my process for the manufacture of carbon electrodes from the mentioned "lamp black", the first of the impurities to be eliminated is the tar.

For this purpose the mass of refuse mat-

ter is subjected to hot water washing and milling, in what is known as a "chaser" mill or wet pan. This operation, which is carried on for a period of approximately 5 twenty minutes agglomerates the tar into pellets about the size of a pea and flat wafers, which is separated by washing in a screen of suitable mesh. The resultant product is finely divided lamp black, which 10 is treated for the elimination of soluble ash by any suitable washing apparatus, wherein the washing is done with successive charges of water, each charge being drained off for washing away the soluble ash. The 15 material with the soluble ash eliminated therefrom is then treated in a roaster or drier, wherein it is agitated while subjected to a temperature of approximately 1000 degrees Fahr., for the removal of all moisture 20 and the high volatile hydrocarbons. This roasting operation is continued for approximately three hours, after which the material is in a dry powdered form, but still contains a trace of hydrocarbon volatiles 25 and from five to ten per cent. by weight of occluded air. To eliminate such volatiles and the occluded air, the material is then charged in fire clay muffles and subjected to a bright red heat at a temperature of be- 30 tween 1800 degrees to 2000 degrees Fahr., and subjected to such roasting for approximately eighteen hours. The resultant product is a gray substance partaking of the 35 qualities of a coke of a high degree of purity and also of a lamp black, though not so fine in grain as the latter, containing approximately one quarter of one per cent. of volatile matter and one half per cent. of insoluble ash.

40 I have found that from certain gas plants a refuse "lamp black" is obtainable free from soluble impurities, in which case the process for washing these out may be eliminated. I have also found that in certain 45 cases where it is desirable to have an electrode with a high degree of tensile strength rather than an extreme fineness of grain, a certain portion of the tar may be added before the material is roasted in the fire clay 50 muffles.

55 After the material has become cool it is ground in a suitable mill and reduced to a fine powder, which is run through separators to remove iron particles which may be contained therein and thereafter there is intermixed therewith a suitable quantity of coal tar or coal tar pitch and oil to act as a binder for the placing of the mixture in a plastic condition, and the same is then 60 compressed into cylindrical cakes. These cakes are formed into green carbon sticks, which are baked in the usual manner for forming carbon electrodes.

The carbons produced from the so-called

"lamp black" refuse of the plants manufacturing illuminating gas from petroleum have proved to be more efficient than the carbon electrodes at present in use. 65

Practical experiments have demonstrated that carbons or electrodes manufactured in accordance with the described invention have a current carrying capacity of about 70 ten per cent. (10%) higher than carbons or electrodes as at present manufactured; for example, after a series of experiments cov- 75 ering about six months' time, it was found desirable to reduce the size of the carbons or electrodes from  $\frac{5}{8}$ " standard to  $\frac{3}{4}$ "<sup>1/2</sup>, and when so reduced the cross sectional area of the improved carbon or electrode had equiv- 80 alent properties with other carbons with cross sectional areas about ten per cent. (10%) greater. When the improved carbons or electrodes were in the full size of  $\frac{5}{8}$ ", they would not operate to the best ad- 85 vantage, as they were "underloaded when subject to the conditions which are considered standard for use of  $\frac{5}{8}$ " electrodes."

Another difference in favor of the improved carbon or electrode found to exist 90 over the standard form of carbons or electrodes in general use, probably based upon their ability to carry a high amount of current, is the characteristic which they possess of carrying an arc free from hissing, when 95 subjected to very high currents and with a short air gap between the electrodes, the improved  $\frac{1}{6}$ " in diameter when carrying from 40 to 42 amperes direct current producing a perfectly quiet arc with a short air gap; 100 whereas, under like conditions the standard carbons at present in use cause hissing and often a so-called "mushroom" would form on the lower or negative electrode.

These above mentioned features bearing 105 upon both the current carrying capacity of the carbon or electrode and upon its production of a quiet arc, under difficult and unusual conditions, are of extreme importance in determining the commercial value of the 110 electrode.

Relative to the specific density of the carbons or electrode produced under the present invention, this can be varied over a considerable range at the will of the manufacturer by changing several different and non-essential factors in the process of manufacture, such as fineness of the dust and density of the coal tar or coal pitch. Tests have demonstrated the improved electrode to 115 have from 10% to 20% less porosity than the standard electrodes at this time placed on the market.

Although the invention is applicable for the production of carbon electrodes, still its 125 use up to the present time has been in the form of electrodes for use in projecting machines used in connection with moving pic-

- ture theaters, spot lights, etc. There is no difference, however, in the manufacture in the production of electrodes for use in projecting, except that it is preferable to add 5 suitable fluxing material to the powder before the coal tar or coal pitch is mixed with it. This flux (usually boracic acid) has a property of combining with the small remaining quantity of ash in the electrodes 10 and being fused by heat of the arc into small pellets, which drop, and, therefore, prevent the ash from accumulating in the electrodes and interfering with the arc. However, the use of such a flux is in no way 15 essential and may be dispensed with, either when applied to the production of carbon electrodes for use in electro-chemical industry and dry batteries, or for use in projecting machines.
- 20 The so-called illuminating gas, which is usually the main product of manufacture when refuse "lamp black" is produced, can be used, of course, for other purposes than as an illuminant, that is in gas engines or as 25 a fuel for firing kilns, boilers, etc. It is, therefore, possible and the scope of this invention contemplates such a possibility for the manufacturer of carbon electrodes to produce his own refuse "lamp black," utilizing 30 the illuminating gas produced for the purpose of firing kilns and the generating of the power used in the factory. The advantage of this method of manufacture would be principally a high degree of control over 35 the quantity, and, in a certain degree, over the quality of the refuse "lamp black" produced, for its quality is dependent almost entirely upon the degree of care exercised in preventing its admixture with outside im- 40 purities, whose presence is in no way essential to the process of the manufacture of illuminating gas.
- I am well aware that true "lamp black" has heretofore been utilized in connection 45 with the manufacture of electrodes, and I therefore do not wish to be understood as claiming the use of such material, but, on the contrary, confine the invention to the use of a so-called "lamp black" refuse de- 50 rived from plants manufacturing illuminating gas; and this irrespective as to whether the manufactured gas be utilized for illuminating, heating or power purposes.
- Having thus described the invention what 55 is claimed as new and desired to be protected by Letters Patent is:—
1. As an article of manufacture, a carbon formed from "lamp black" derived from the waste by-products of the manufacture of 60 oil gas, and a carbonaceous binder intermixed therewith.
2. The method of producing carbon electrodes from the refuse "lamp black" product of the manufacture of gas, which consists
- in eliminating from said product foreign 65 impurities, thence forming the material into a plastic body, thence producing green sticks therefrom and finally baking said sticks for the production of carbon electrodes.
3. The method of producing carbon elec- 70 trodes from the lamp black refuse derived from the manufacture of gas from oil, which consists first in eliminating therefrom by washing the tar contained therein, thence removing the soluble ash, thence roasting 75 under agitation for the removal of moisture and the high volatile hydrocarbons, thence roasting at a higher temperature for the elimination of remaining hydrocarbons, thence reducing the material to a powder, 80 adding thereto a suitable flux and forming the whole into a plastic body, thence forming the same into green carbon sticks and finally baking the same for the production 85 of the required carbon electrodes.
4. The method of producing carbon electrodes from lamp black refuse derived from the manufacture of gas from oil, which consists first in eliminating from the material by washing and roasting the impurities con- 90 tained therein, thence forming the material into a plastic body, thence producing green sticks therefrom and finally baking said sticks for the production of carbon elec- 95 trodes.
5. The method of producing carbon electrodes from lamp black refuse derived from the manufacture of gas from oil, which consists first in eliminating from the material by washing and roasting the impurities con- 100 tained therein, thence reducing the material to a powder having incorporated therein a suitable flux, then forming the material into a plastic body and producing therefrom green sticks, and finally baking said sticks 105 for the production of the carbon electrodes.
6. The method of producing carbon elec- 110 trodes which consists in separating from the carbonaceous refuse product of gas manu- 115 facture the tar, hydrocarbons and moisture contained therein, reducing the resultant refuse "lamp black" to powdered form, thence forming the same into a plastic body and producing therefrom green sticks, and finally baking said sticks for the production of electrodes.
7. The method of producing carbon elec- 120 trodes which consists in removing from the waste by-products of gas manufacture the tar, volatile hydrocarbons, and water, re- 125 ducing the resultant product thereof into a powder, intermixing therewith a suitable binder for placing the same in a plastic condition, thence forming therefrom green sticks, and finally baking said sticks for the production of electrodes.
8. The method of producing carbon elec- 130 trodes, which consists in separating the

volatiles from the waste by-products of the manufacture of oil gas for the recovery therefrom of the so-called "lamp black", reducing the same to a finely divided condition, intermixing therewith a carbonaceous binder, and thence baking the same for the production of carbons.

In testimony whereof I have signed my name to this specification in the presence of two subscribing witnesses.

ROBERT D. PIKE.

Witnesses:

N. A. ACKER,  
D. B. RICHARDS.